

## UNITED STATES PATENT OFFICE

2,167,684

## ALLOY

Charles B. Sawyer, Cleveland Heights, Ohio, assignor to The Brush Beryllium Company, Cleveland, Ohio, a corporation of Ohio

No Drawing. Application February 15, 1937,  
Serial No. 125,817

4 Claims. (Cl. 75—159)

The invention relates to alloys composed predominantly of copper, and has to do especially with an improved alloy containing copper, beryllium and nickel.

5. Copper-beryllium alloys are characterized by their susceptibility to precipitation hardening effected by suitable heat treatment, such alloys containing from about 1% to 10% by weight of beryllium being susceptible to such treatment.  
10 Such alloys containing 2% and upwards of beryllium have some excellent qualities but are not sufficiently susceptible to working to make them well suited for some uses. Also such copper-beryllium alloys, in the heat hardened state  
15 are subject to softening when subjected in use to elevated temperatures.

I have discovered that it is possible by the addition to such copper-beryllium mixtures containing upwards of 2% to about 8% of beryllium 20 of suitable amounts of nickel, ranging upwards of 1% to about 8% and preferably from 1.25% to 5.0%, to produce alloys having working properties notably superior to the corresponding copper-beryllium alloys, substantially higher hardness (Brinell) in the heat hardened state and the ability, in the heat hardened state, to withstand elevated temperatures about fifty degrees higher than can the corresponding copper-beryllium alloys. Furthermore, the tensile strength 25 and elongation under tensile stress of my improved alloys are at least equal to the corresponding copper-beryllium alloys. Nor do my new alloys show substantial impairment of electrical conductivity as compared with the copper-beryllium alloys. The new alloys are also characterized by excellent casting properties, castings made from them being distinguished by unusual soundness and a fine grain structure 30 whereas no little difficulty has heretofore been had in the production of sound castings from copper-beryllium alloys. The properties of my copper-beryllium-nickel alloys naturally vary within the composition limits of upwards of 2% to 8% beryllium and upwards of 1% to 8% nickel. 35 Alloys ranging upwards of 2% to 3% beryllium and 1.25% to 5% nickel have a desirable combination of properties fitting them for many different uses and, generally speaking, I consider this range of compositions as preferable.  
40 In the preparation of the new alloys it is convenient to have on hand copper-beryllium master alloy which may range from 3% to 10% beryllium content. Since nickel dissolves slowly in copper, it is also desirable to have available  
45 a copper-nickel alloy containing from 10% to  
50

40% of nickel. Pure copper is also required. The relative components are first weighed out, with an allowance of 5% to 10% for loss of beryllium by oxidation during alloying. The copper and the copper-nickel alloy are then melted together and the copper-beryllium alloy is added last. A clay and graphite crucible may be used. The lowest pouring temperature possible should be used in order to avoid porosity in the casting.

5 After casting, the alloy may be forged, or heat treated directly without forging. The best temperature for forging is about 750° C.—780° C.

The heat treatment for the production of precipitation hardening suitable for the new alloys consists of the two steps of quenching from a 15 suitable elevated temperature and reheating at a lower temperature, the treatment being of the same general character employed for the precipitation hardening of copper-beryllium alloys but differing somewhat as to the preferred temperatures employed. The first step consists in heating the alloy to a temperature high enough to bring all or most of the beryllium into solid solution, a temperature of about 830° C. being suitable. This is somewhat higher than the temperature most suitable in the case of plain copper-beryllium alloys. After this initial heating which may last as much as two hours at the maximum temperature, the alloy is quickly quenched so as to retain the various components 20 in the solid solution into which they have been more or less entirely transformed by the heating. The longer the exposure to the maximum temperature, the more complete is the solution. After quenching from the elevated temperature 25 the material is reheated to a temperature of 300° C. to 350° C. to effect the precipitation hardening. The time of exposure to the lower or hardening temperature may be varied widely, depending upon the properties desired, the temperature employed, and the degree and kind of working previously performed on the alloy. While I have mentioned the preferred range of temperature as 300° C. to 350° C., higher and lower temperatures may be employed. The specified range of temperature, it may be noted, is about fifty degrees higher than that most suitable for plain copper-beryllium alloys.

The presence of nickel in my alloys retards the precipitation of the hardening component 50 so that the rate of cooling from the high temperatures, during the initial step of the hardening treatment, does not need to be so high. This is of advantage in hardening large cross sections for which the ratio of surface to mass is low, 55

with corresponding difficulty in extracting the heat quickly even with water quenching. For thin cross sections where the ratio of surface to mass is high, it becomes increasingly possible to 5 use air quenching, while moderate sized sections can be quenched in oil as has been found preferable in hardening steel, when minimum deformation is demanded. This feature is of especial 10 value in the case of castings. Furthermore, in the re-heating to effect hardening, the presence 15 of nickel in my alloys makes the exact time of reheating at any given temperature much less critical than for plain copper-beryllium alloys, the danger of softening the nickel alloy by too long exposure being reduced.

I have found that a more homogeneous structure is obtained after hardening, if the alloy has first been subjected to hot or cold working. With 20 this in view, such working may advantageously be effected between the initial quenching from high temperature and the subsequent final heat treatment to effect hardening.

As an example of the improved properties which 25 characterize the new alloys, a copper-beryllium alloy containing 2.39% beryllium had maximum Brinell hardness, in the hardened state, of 375 while an alloy with substantially the same (2.38%) beryllium content and 1.98% nickel content had a Brinell hardness of 387. The plain 30 beryllium-copper alloy attained its maximum hardness by re-heating for two hours at 300° C. but when heated to the same temperature for twenty hours its Brinell hardness dropped to 290 and a further heating for six hours at 330° C. 35 caused its Brinell hardness to drop further to 269. On the other hand, the copper-beryllium-nickel alloy withstood the same entire treatment without any reduction of its hardness and the same alloy when subjected to a temperature of 330° 40 for twenty-six hours after reaching its maximum Brinell hardness of 387 suffered only the slight reduction in hardness to 381. The increase in Brinell hardness resulting from the addition of nickel to copper-beryllium alloys containing upwards of 2% beryllium may run as high 45 or higher than 40 points.

The improved properties of my alloy are also outstanding in comparison with prior ternary alloys of copper, beryllium and nickel. An alloy 50 of my invention composed of 2.3% beryllium, 1.1% nickel, 0.1% iron and the remainder copper, in rolled sheet form, showed a maximum tensile strength of 211,000 pounds per square inch and 2% elongation, in comparison with 193,000 pounds 55 per square inch and 2% elongation for an alloy in rolled sheet form containing about 2.25% beryllium, about 0.5% nickel, about 0.1% iron and balance copper. Also, the second of these two alloys has a proportional limit of 55,000 pounds 60 per square inch, whereas my improved alloys have proportional limits varying from 75,000 pounds per square inch to 100,000 pounds per square inch. My improved alloys have electrical conductivities fully as high as that of the above 65 alloy having 0.5% nickel, when both alloys have been heat treated to give their maximum mechanical properties. The foregoing proportional limit values were determined on specimens of two inches gauge length.

70 The fields of use for which my improved alloys are especially adapted are more or less indicated by what has been said about the properties of the alloys and the characteristics of their hardening treatment. The soundness and fine grain structure on casting and the latitude as to rate of

cooling and length of exposure to heat in the heat treating steps especially adapt the new alloys to use for the production of castings. Obviously, the marked extent to which the new alloys are susceptible of working well adapt the alloys for 5 the production of forgings and products otherwise subjected to working in their production. The resistance of the alloys to elevated temperatures without loss of hardness makes them especially adapted for such uses as dies, molds for 10 the casting of metals and the formation of plastics, welding electrodes, turbine blades, electrical contacts, and springs required to operate at elevated temperatures. My alloys also are highly 15 resistant to abrasion.

Metallographic sections of my improved alloys quenched from temperatures ranging upward from about 800° C. to near their melting points, show an unusual metallographic phase. This 20 part may be quite visible after polishing and without etching, appearing as a much harder phase of the alloy. Its frequently dendritic form suggests separation at a high temperature, though it readily changes to a globular form. The usual alpha phase of copper-beryllium alloys is always present 25 and the known beta phase of such alloys may also be present, depending upon the relative amounts of nickel and beryllium used. Since the new phase appears in greater quantities with increase in nickel and beryllium contents, quite 30 possibly it is a combination of nickel and beryllium, with or without copper, which forms the precipitation hardening agent appearing in these 35 alloys in the alpha and beta phases on re-heating. Whether it replaces the customary hardening phase of plain beryllium copper or appears in addition to it, is not now certain, nor is it known whether the new phase may itself decompose on 40 re-heating. In any event, it appears that these new alloys show a distinctive metallographic 45 phase.

Increase in nickel content above 1% with corresponding increase in the new metallographic phase seems to militate against the occurrence 50 of the beta phase often found in beryllium-copper quenched from about 800° C. or above. Such beta phase in alloys of 2% to 2.5% beryllium quenched from 800° C. and above, would not be expected from the latest of the known published beryllium-copper equilibrium diagrams and where 55 such beta phase occurred in prior investigations it was commonly believed to occur because of lack of equilibrium in the alloys. I have found, however, that at the above temperature, the beta phase is a normal equilibrium phase in binary 60 alloys having more than about 2% beryllium. The effect of adding nickel to beryllium-copper alloys containing more than about 2% of beryllium is to cause the beta phase to disappear wholly or in part, or possibly to replace it with the new 65 phase. This is apparent with more than 1% added nickel and quite marked with 2% added nickel. The advantages of my new alloy are believed to spring from the characteristics of the new phase as well as from the suppression of the beta phase. I note especially that the new phase is dispersed within the grains in small globular particles instead of being located at the grain boundaries in relatively large angular particles as is the case with the beta phase. The globular 70 form and dispersed distribution of the new phase are advantageous in suppressing grain growth without the attendant weakening of the whole alloy which often proceeds from the inclusion of the beta phase at the grain boundaries of the 75

alpha phase. Such weakening is especially marked in drawn alloys containing the hard beta phase since the drawing of such alloys may produce minute internal fractures which lower their endurance limits.

In my experience commercial beryllium-copper, nickel, and copper always contain some impurities such as iron, aluminum, silicon, cobalt, and zinc. While these elements undoubtedly have a small effect on the resulting alloy, in defining my improved alloys as composed of copper, beryllium and nickel I do not mean to exclude such other elements in any amounts insufficient substantially to alter the characteristic properties of the alloys. Commercial beryllium-copper generally contains iron in the neighborhood of 0.1% and may reach an amount as great as 0.35%; silicon may be present from 0.03% to 0.1%; nickel generally contains 1% cobalt, while "high grade" copper may contain up to a total of 0.1% of several impurities including zinc. Lead and antimony are deleterious even in very small amounts. Aluminum is present with beryllium in amounts ranging from

0.01% to 0.2% depending on the efficiency of its separation from beryllium.

What I claim is:

1. A copper base alloy containing beryllium in an amount within the range of upwards of 2% to 6% and which would cause the presence of the known beryllium-copper beta equilibrium phase if the binary combination is quenched from a temperature of 800° C.; nickel in an amount within the range of upwards of 1% to 8% and which is effective substantially to suppress the said beta phase; and the remainder substantially all copper.
2. An alloy as claimed in claim 1, wherein the beryllium is upwards of 2% to 3%, and the nickel content is from about 1.25% to 5%.
3. An alloy containing from substantially 2.25% to 6% of beryllium, upwards of 1% to 8% of nickel, with the remainder substantially all copper.
4. An alloy containing from substantially 2.25% to 3% of beryllium and from 1.25% to 5% nickel, with the remainder substantially all copper.

CHARLES B. SAWYER.

CERTIFICATE OF CORRECTION.

Patent No. 2,167,684.

August 1, 1939.

CHARLES B. SAWYER.

It is hereby certified that error appears in the printed specification of the above numbered patent requiring correction as follows: Page 2, second column, line 20, for the word "part" read phase; line 21, for "phase" read part; and that the said Letters Patent should be read with this correction therein that the same may conform to the record of the case in the Patent Office.

Signed and sealed this 5th day of September, A. D. 1939.

(Seal)

Henry Van Arsdale,  
Acting Commissioner of Patents.

alpha phase. Such weakening is especially marked in drawn alloys containing the hard beta phase since the drawing of such alloys may produce minute internal fractures which lower their endurance limits.

In my experience commercial beryllium-copper, nickel, and copper always contain some impurities such as iron, aluminum, silicon, cobalt, and zinc. While these elements undoubtedly have a small effect on the resulting alloy, in defining my improved alloys as composed of copper, beryllium and nickel I do not mean to exclude such other elements in any amounts insufficient substantially to alter the characteristic properties of the alloys. Commercial beryllium-copper generally contains iron in the neighborhood of 0.1% and may reach an amount as great as 0.35%; silicon may be present from 0.03% to 0.1%; nickel generally contains 1% cobalt, while "high grade" copper may contain up to a total of 0.1% of several impurities including zinc. Lead and antimony are deleterious even in very small amounts. Aluminum is present with beryllium in amounts ranging from

0.01% to 0.2% depending on the efficiency of its separation from beryllium.

What I claim is:

1. A copper base alloy containing beryllium in an amount within the range of upwards of 2% to 6% and which would cause the presence of the known beryllium-copper beta equilibrium phase if the binary combination is quenched from a temperature of 800° C.; nickel in an amount within the range of upwards of 1% to 8% and which is effective substantially to suppress the said beta phase; and the remainder substantially all copper.
2. An alloy as claimed in claim 1, wherein the beryllium is upwards of 2% to 3%, and the nickel content is from about 1.25% to 5%.
3. An alloy containing from substantially 2.25% to 6% of beryllium, upwards of 1% to 8% of nickel, with the remainder substantially all copper.
4. An alloy containing from substantially 2.25% to 3% of beryllium and from 1.25% to 5% nickel, with the remainder substantially all copper.

CHARLES B. SAWYER.

CERTIFICATE OF CORRECTION.

Patent No. 2,167,684.

August 1, 1939.

CHARLES B. SAWYER.

It is hereby certified that error appears in the printed specification of the above numbered patent requiring correction as follows: Page 2, second column, line 20, for the word "part" read phase; line 21, for "phase" read part; and that the said Letters Patent should be read with this correction therein that the same may conform to the record of the case in the Patent Office.

Signed and sealed this 5th day of September, A. D. 1939.

(Seal)

Henry Van Arsdale,  
Acting Commissioner of Patents.